

## UNITED STATES PATENT OFFICE.

MORRIS C. VAN GUNDY, OF PORT ARTHUR, TEXAS, ASSIGNOR TO THE TEXAS COMPANY, OF NEW YORK, N. Y., A CORPORATION OF TEXAS.

## LUBRICATING COMPOUND.

No Drawing.

Application filed December 11, 1920. Serial No. 430,040.

To all whom it may concern:

Be it known that I, MORRIS C. VAN GUNDY, a citizen of the United States, residing in Port Arthur, in the county of 5 Jefferson and State of Texas, have invented certain new and useful Improvements in Lubricating Compounds, of which the following is a specification.

This invention relates to the formation of 10 solid lubricating compounds intended primarily for use on heavy bearing surfaces, such for example as driving journals.

It is common practice to prepare lubricating compounds by mixing a mineral and 15 fatty oil and saponifying with caustic soda. I have discovered that the admixture of a small quantity of lead soap to the compound increases the lubricating value of the product and forms a lubricant particularly 20 adapted for lubricating heavy bearings.

In accordance with my invention I employ suitable portions of alkali soap such as soda soap, mineral oil and a small portion of lead soap, ordinarily about 10%.

25 As a specific example of the invention I may give the following:

|                                    |        |
|------------------------------------|--------|
| Fatty oil (e. g. tallow) -         | 40.00% |
| Alkali (e. g. caustic soda) -      | 8.00%  |
| Lead soap -----                    | 10.00  |
| Mineral oil (cylinder stock) ----- | 32.75  |
| Water -----                        | 9.25   |

The proportion of lead soap used will depend upon the particular use for which the compound is intended. For the preparation of a solid lubricating cake, however, the proportion will not ordinarily exceed 20% and will generally be around 10%.

Any suitable mineral oil may be employed 40 in the preparation of the compound. In the example given above a paraffin cylinder stock was used but the mineral oil content may comprise a mixture of paraffin lubricating stock and an asphaltic residue such as 45 flux oil.

What I claim is:-

1. A lubricant comprising an alkali soap, a mineral oil, and lead soap which in quantity constitutes approximately 10% of the 50 compound.

2. A lubricant comprising approximately

40%—Fatty oil,  
8%—Caustic soda,  
10%—Lead soap,  
33%—Mineral oil,  
9%—Water.

3. A lubricant comprising a petroleum 60 cylinder stock admixed with an alkali soap and a lead soap which in quantity constitutes approximately 10% of the compound.

In witness whereof I have hereunto set my hand this 1st day of December, 1920.

MORRIS C. VAN GUNDY.